

## UNITED STATES PATENT OFFICE

ARCHIE B. HOEL, OF DREXEL HILL, PENNSYLVANIA, ASSIGNOR TO THE ATLANTIC  
REFINING COMPANY, OF PHILADELPHIA, PENNSYLVANIA, A CORPORATION OF  
PENNSYLVANIA

## EMULSIFIABLE OIL AND METHOD OF PRODUCING SAME

No Drawing.

Application filed May 24, 1929. Serial No. 365,779.

The present invention relates to emulsifiable oils, as for example, of the type known as "cutting" oil, or oils to be used in the textile industry or the like.

5 An oil prepared in accordance with my invention is an improved product over known emulsifiable oils in that when dissolved in water a substantially non-frothing emulsion is formed.

10 In accordance with prior practice, oils used in forming mineral oil emulsions are usually prepared by mixing a suitable emulsifying agent, as for example, soaps formed from rosin, fatty acids, sulphonated vegetable or animal oil, or certain acids derived from petroleum, or a mixture of them, with mineral oil, preferably a light lubricating hydrocarbon oil. Such oils when agitated with water have the tendency to form a more 20 or less persistent froth or foam. This frothing or foaming tendency is highly undesirable, one reason being that it causes overflowing of the vats or tanks in which the emulsion is made up. An object of my invention is to produce an oil which during or 25 after its formation of an emulsion with water will not give a persistent froth when agitated.

I have found that when sulphonated sperm 30 oil or a similar liquid wax is compounded with mineral oil and saponified either before or after such compounding, there is formed a product which when agitated with water has little or no frothing tendency. Furthermore, I have found that when sulphonated sperm oil is compounded with mineral oil and any of the commonly known emulsifying agents, such as rosin, fatty acids, 35 sulphonated vegetable or animal oil, or the like, and the mixture is saponified and thereafter emulsified with water, there is produced an emulsion which has little or no frothing tendency when agitated.

40 In the preparation of an emulsifiable oil in accordance with my invention, I take a suitable hydrocarbon oil, as for example, one having a saybolt viscosity at 100° F. of from 100 to 200 seconds or even higher, preferably 45 an oil of the light lubricating class, and add

thereto sulphonated sperm oil and an alkali, each of the last two ingredients in sufficient amounts so that the final product will readily emulsify when water is added thereto. The product resulting is an emulsifiable oil which is clear, homogeneous and non-gelatinous, and in forming an emulsion with water will not form a persistent froth or foam, nor will the emulsion after having been formed, froth or foam to any substantial extent when agitated. Furthermore the emulsion so formed will be a practically perfect and permanent milk white liquid.

55 For a portion of the sulphonated sperm oil used in forming my emulsifiable oil there 60 may be substituted other emulsifying agents, as for example, rosin, fatty acids, sulphonated vegetable and/or animal oils, certain sulphonated acids derived from petroleum, or the like. Such emulsifying agents may be 65 either added to the sulphonated sperm oil and the mixture added to mineral oil or the sperm oil and additional emulsifying agent may be added to the mineral oil separately; 70 whereupon an amount of alkali sufficient to 75 effect the desired saponification is added thereto.

80 It is to be understood that there are limits within which sulphonated sperm oil as such or with an additional emulsifying agent 85 may be compounded with mineral oil to produce a satisfactory emulsifiable oil. If too little sulphonated sperm oil or too little of the mixture of emulsifying agents is added, the product resulting will not be completely soluble in water or in other words will not 90 form a satisfactory emulsion, while if too much of the sulphonated sperm oil or the mixture is added the product will froth or foam when an emulsion with water is formed. Also, if the mixture of emulsifying agents is used and there is insufficient sulphonated sperm oil in the mixture the product may 95 froth or foam when an emulsion is made therewith. In general, the amount of sulphonated sperm oil or mixture of sulphonated sperm oil and additional emulsifying agent used will depend upon the particular mineral oil to which it is to be added and in the mixture the amount of sulphonated 100

sperm oil used will depend upon the properties of the particular emulsifying agent mixed therewith, therefore I do not contemplate limiting my invention to any specific percentages of ingredients.

As an example of a method whereby an emulsifiable oil which when mixed with water will form a non-frothing stable emulsion may be prepared in accordance with my invention, 10 but without intending to be limited thereby, I may add about 80 parts of mineral oil preferably a light lubricating oil, to about 20 parts of sulphonated sperm oil and agitate either mechanically or otherwise until the 15 oils are thoroughly mixed, then slowly add to the mixture while continuing the agitation, a caustic potash solution, as for example, a 38° Bé. solution, in sufficient amounts to produce the desired saponification, which will be evidenced by the oil becoming clear and transparent, and completely emulsifiable with water.

As a further example, using an additional emulsifying agent, in this particular case, 20 rosin, I first put into a kettle about 50 parts by weight of the rosin and melt it. The rosin used should be preferably of a good grade of light colored wood or gum rosin and should melt at around 185° F. To the melted rosin I 25 add about 625 parts by weight of a light lubricating mineral oil and mix the whole thoroughly. Then with the temperature of the mixture around 150° F., I add thereto about 125 parts by weight of sulphonated sperm oil, 30 and agitate for several minutes. I then add about 16 parts by weight of a 40° Bé. potassium hydroxide solution very slowly, at the same time agitating so that saponification 35 will be effected. The finished oil will when 40 mixed with water produce a non-frothing stable emulsion.

It is to be understood that the essential feature of my invention comprises the addition of sulphonated sperm oil or a similar 45 liquid wax to mineral oil for the purpose of producing an emulsifiable oil which when mixed with water will form a non-frothing stable emulsion for use as heretofore described. It is to be further understood that 50 any alkali which causes saponification of the saponifiable constituents in the mixture may be used in preparing my product, and that either one or more of the emulsifying agents which are well known to those skilled in the 55 art may be added to or substituted for a part of the sulphonated sperm oil, for the production of an emulsifiable oil in accordance with my invention.

Herein the term "non-foaming emulsifiable oil" refers to an oil which when mixed with water to produce an emulsion, will form such emulsion without the usual persistent froth or foam which is incident to the formation of emulsions with emulsifiable oils containing mineral oil now in common use. It

is not meant to convey that an emulsion formed by mixing or agitating my oil with water will not foam at all, but that such small amount of foam as may form will not persist, or in other words, will subside immediately whereupon there will be no head of foam upon the emulsion.

What I claim is:

1. The process which consists in mixing mineral oil with saponified sulfonated sperm oil to produce a clear, homogeneous, non-gelatinous emulsifiable oil, and mixing the emulsifiable oil with water to form a non-frothing stable emulsion.

2. The process which consists in mixing a relatively small amount of sulfonated sperm oil with a relatively large amount of mineral oil, then agitating and adding an alkali in sufficient quantities to at least partially saponify the sulfonated sperm oil, thereby to produce a clear, homogeneous, non-gelatinous emulsifiable oil, and mixing the emulsifiable oil with water to form a non-frothing stable emulsion.

3. The process which consists in mixing saponified sulfonated sperm oil, an additional emulsifying agent and mineral oil, thereby to produce a clear, homogeneous, non-gelatinous emulsifiable oil, and mixing the emulsifiable oil with water to form a non-frothing stable emulsion.

4. The process which consists in mixing sulfonated sperm oil, an additional emulsifying agent and mineral oil, then agitating and adding an alkali in sufficient quantities to at least partially saponify the sulfonated sperm oil, thereby to produce a clear, homogeneous, non-gelatinous, emulsifiable oil, and mixing the emulsifiable oil with water to form a non-frothing stable emulsion.

5. The process which comprises mixing sulfonated sperm oil, mineral oil and one or more emulsifying agents from the group comprising rosin, fatty acids, sulfonated vegetable oil, and acids derived from petroleum, then agitating and adding an alkali in sufficient quantities to at least partially saponify the saponifiable material present in the mixture, thereby to produce a clear, homogeneous, non-gelatinous emulsifiable oil, and mixing the emulsifiable oil with water to form a non-frothing stable emulsion.

6. The process which comprises mixing mineral oil with a quantity of saponified sulfonated sperm oil sufficient to amount to at least 15 per cent of the total mixture, thereby to produce a clear, homogeneous, non-gelatinous emulsifiable oil, and mixing the emulsifiable oil with water to form a non-frothing stable emulsion.

7. The process which consists in mixing mineral oil, saponified sulfonated sperm oil, and an additional emulsifying agent in proportions so that at least 15 per cent of the total mixture will be saponified sulfonated

sperm oil, thereby to produce a clear, homogeneous, non-gelatinous emulsifiable oil, and mixing the emulsifiable oil with water to form a non-frothing stable emulsion.

5 8. The process which comprises forming a mixture of mineral oil and saponified sulfonated sperm oil containing at least 15 per cent of the latter, and agitating said mixture with water, thereby to produce a non-frothing stable emulsion.

10 9. The process which consists in mixing mineral oil, saponified sulfonated sperm oil and an additional emulsifying agent, then agitating the mixture with water, the saponified sulfonated sperm oil being present in sufficient quantities so that the emulsion formed will be stable and non-frothing.

15 10. The process which comprises mixing mineral oil, sulfonated sperm oil and one or 20 more emulsifying agents from the group comprising rosin, fatty acids, sulfonated vegetable oil, and acids derived from petroleum, then adding sufficient alkali to at least partially saponify the saponifiable materials 25 present, then agitating the mixture with water, thereby to produce a non-frothing stable emulsion.

30 11. A clear, homogeneous, non-gelatinous, emulsifiable oil consisting of mineral oil and saponified sulfonated sperm oil.

35 12. A clear, homogeneous, non-gelatinous, emulsifiable oil consisting of mineral oil, saponified sulfonated sperm oil and one or more emulsifying agents from the group comprising rosin, fatty acids, sulfonated vegetable oil, and acids derived from petroleum.

40 13. A non-frothing stable emulsion of water and oil which consists of mineral oil, saponified sulfonated sperm oil and water.

45 14. A non-frothing stable emulsion which consists of a mixture of mineral oil, saponified sulfonated sperm oil, one or more emulsifying agents from the group comprising rosin, fatty acids, sulfonated vegetable oil, and acids derived from petroleum, and water.

In testimony whereof I affix my signature.

ARCHIE B. HOEL.

50

55

60

65